

## UNITED STATES PATENT OFFICE

2,339,545

## METHOD OF PLATING POLONIUM

John H. Dillon, Akron, Ohio, assignor to The Firestone Tire & Rubber Company, Akron, Ohio, a corporation of Ohio

No Drawing. Application October 21, 1940,  
Serial No. 362,061

3 Claims. (Cl. 117—62)

This invention relates to the art of plating polonium and relates especially to a method of removing surface impurities from a metal plated with polonium.

Polonium is a radioactive metal classified in the uranium-radium family of radioactive elements. It has a half-life period of about 138 days and is a powerful emitter of strong alpha rays. It emits practically no beta rays or gamma rays, and, during the course of its relatively short life it gradually changes directly into an inactive isotope of lead. By virtue of its unique properties polonium is utilized, both scientifically and commercially, as a convenient and efficient agent for ionizing gases. An example of an important commercial use of polonium is the incorporation of an extremely small amount of the metal in an internal combustion engine spark plug near the spark gap thereof for the purpose of substantially improving the sparking characteristics of the plug.

Polonium occurs in commercially significant quantities in radio-lead compounds which are a by-product of the radium refining industry. Radio-lead, consists mainly of lead, but contains small amounts of radium D and polonium. The usual commercial process of isolating polonium comprises forming a solution of a soluble salt, preferably the chloride, of radio-lead and then plating the polonium from this solution onto another metal. Electroplating with applied voltage is not necessary, as the polonium will plate onto most other metals by adsorption or chemical displacement. According to a preferred procedure polonium is plated by chemical displacement from a hot solution of radio-lead chloride onto nickel foils. The plated nickel foils may be used directly, melted with or without the addition of other metal to form a polonium alloy, or treated to drive off the free polonium (e. g., by vaporization) so that it may thereafter be isolated in a more concentrated form.

The radio-lead chloride for the plating solution is generally prepared by treating radio-lead oxide with hydrochloric acid. Freshly prepared radio-lead chloride usually contains a slight amount of the unconverted lead oxide in a very finely divided form. When such fresh preparation is used in a polonium plating bath, the finely divided oxide deposits mechanically on the metal being plated. The polonium is distributed throughout the lead oxide scale on the surfaces of the metal. Since lead is considered very objectionable in nickel and other alloys, from the standpoint of the processing and the physical proper-

ties thereof, it is desirable to remove this lead oxide from the plated metal without appreciable loss of polonium therefrom, if the metal is to be thereafter incorporated in an alloy.

It is, therefore, a primary object of the invention to provide a practical method of removing surface impurities from a polonium plated metal without substantial loss of polonium therefrom.

Another object is to provide a method of treating a polonium-plated metal to render it capable of taking up a further quantity of polonium in a subsequent plating operation.

The above and further objects will be apparent in the description of the invention which follows.

The invention comprises treating polonium-plated metal with nitric acid of a certain strength in order to remove therefrom undesired surface impurities, such as lead oxide, without substantial loss of polonium from the metal. It has been discovered that a treatment of polonium-plated metal containing lead oxide with ordinary concentrated nitric acid containing about 70 per cent of  $\text{HNO}_3$  removes all of the lead oxide together with most of the polonium. On the other hand, when such metal is treated with a nitric acid containing less than about 35 per cent of  $\text{HNO}_3$ , all of the lead oxide is not removed, although there is no loss of polonium. Treatment of the metal with acid containing about 35 to 40 per cent of  $\text{HNO}_3$  completely removes the lead oxide from the plated metal without occasioning the loss of a substantial quantity of the polonium therefrom.

The following examples are presented for the purpose of illustrating specific applications of the invention and are not meant to be construed as limiting the invention thereto.

## EXAMPLE I

Nickel foils were plated with polonium by immersion in a boiling solution of radio-lead chloride, freshly prepared from radio-lead oxide. The plated foils were uniformly pink, because of the lead oxide precipitated thereon from the plating solution. The polonium contents of the foils were determined by a known method of measuring the alpha ray emission of the foils, and then several foils were separately immersed in nitric acid of a definite strength for a short time. Thereafter the foils were rinsed with water, dried, and examined for freedom from lead oxide (freedom from any pink appearance) and for any loss in polonium content. Table I shows the results obtained with various concentrations of  $\text{HNO}_3$ , made up by adding 100 parts by volume of con-

centrated nitric acid to various volumes of water, as indicated.

Table I

| Volume concentrated acid to water | Per cent HNO <sub>3</sub> | Immersion time       | Per cent loss of polonium | Removal of lead oxide |
|-----------------------------------|---------------------------|----------------------|---------------------------|-----------------------|
| 100/0.....                        | 70                        | Instantaneous.....   | 87                        | Complete.             |
| 100/100.....                      | 41                        | .....do.....         | 20                        | Do.                   |
| 100/125.....                      | 37                        | 30 seconds.....      | 3.6 to 6.7                | Do.                   |
| 100/150.....                      | 34                        | 6 to 60 seconds..... | 0                         | Not quite complete.   |

It is apparent from Table I that 34 per cent HNO<sub>3</sub> is unsatisfactory, since it does not completely remove the lead oxide. The 70 per cent HNO<sub>3</sub> (ordinary concentrated nitric acid) is manifestly too concentrated, since it removes most of the polonium from the foils. The 37 per cent acid is a practical compromise, since it removes all of the lead oxide without removing much polonium. The 41 per cent acid is near the upper practical limit, in that it occasions the loss of about 20 per cent of the polonium. Therefore, a range of about 35 to about 40 per cent HNO<sub>3</sub> is preferred for treating the foils.

## EXAMPLE 2

Polonium-plated foils with surfaces contaminated with lead oxide were cleaned by immersion in approximately 37 per cent nitric acid, in the manner set out in Example 1. Table II shows the change in the apparent polonium content of the foils after treatment.

Table II

| Immersion time   | Change in apparent polonium content |
|------------------|-------------------------------------|
| 30 seconds.....  | 4.60% loss.                         |
| 30 seconds.....  | 7.95% gain.                         |
| 180 seconds..... | 8.10% gain.                         |

The apparent gain in polonium content of certain foils cleaned by immersion in the nitric acid bath can be readily explained on the assumption that both the lead oxide and the surface polonium initially dissolve in the nitric acid, and then most of the dissolved polonium re-plates onto the cleaned foil surface. Since there is no longer any lead oxide present as a scale on the surface of the foil to absorb some of the alpha rays emitted by underlying polonium, a higher apparent polonium content may be indicated on measuring the alpha ray emission of the cleaned foil.

## EXAMPLE 3

Nickel foils were polonium-plated in the manner described in Example I and then cleaned of lead oxide by immersion in approximately 37 per cent nitric acid for 30 seconds. The foils were rinsed thoroughly with water and then placed in a fresh radio-lead chloride plating bath for a second plating. After the usual plating period the foils were examined and found to have approximately double the polonium content of foils plated only once. Plated foils contaminated with lead oxide, and not cleaned with nitric acid as above, were found to increase only slightly in polonium content on being subjected to a second plating operation.

The successfully double-plated foils may be cleaned a second time by immersion in nitric acid of the strength designated above, and thereafter, if desired, subjected to a third plating operation to increase their polonium content substantially. Thus, foils having exceptionally high surface polonium contents are readily prepared for special uses by the application of two or more plating operations thereto.

The cleaning period is judged by the appearance of the foils before and after immersion in the acid. Usually the oxide scale is pink, but occasionally it has a black or bluish cast. Ordinary plated foils, having a light pink cast, are completely cleaned by immersion for about 5 to 30 seconds in the nitric acid, whereas foils having a heavy deposit of oxide may require immersion for as long as about three minutes. Modification may be resorted to without departing from the scope and spirit of the invention as set forth in the appended claims.

What is claimed is:

1. The method of removing surface lead oxide from polonium-plated metal which comprises treating the plated metal with approximately 37 per cent aqueous nitric acid.
2. The method of removing surface lead compounds from polonium-plated metal which comprises treating the plated metal with 35 to 40 per cent aqueous HNO<sub>3</sub>.
3. The method of producing polonium-plated metal having an exceptionally high surface concentration of polonium which comprises the steps of plating polonium from a solution containing the same onto a metal, then treating the plated metal with 35 to 40 per cent aqueous HNO<sub>3</sub>, and thereafter plating a further quantity of polonium onto the plated metal.